

3,808,134

## SYNTHETIC HYDROCARBON LUBRICANT COMPOSITIONS

Hugh Ernest Romine, Ponca City, Okla., assignor to  
 Continental Oil Company, Ponca City, Okla.  
 No Drawing. Filed Aug. 9, 1972, Ser. No. 280,059  
 Int. Cl. C10m 1/28

U.S. Cl. 252—59

11 Claims

## ABSTRACT OF THE DISCLOSURE

Compositions comprising mixtures of di-n-alkaryl (e.g., di-n-alkylbenzenes) and linear mono-olefin oligomers have certain improved properties over that of either alone. For example, mixtures of the two materials have a lower —40° F. viscosity, as compared to the interpolated viscosity, than either material alone. Also, mixtures of the two materials are more compatible to additive combinations than the linear mono-olefin oligomer alone. Still further, compositions comprising the mixtures and various additive combinations have improved viscosity indexes as compared to either material containing the additive package.

## BACKGROUND OF THE INVENTION

## Field of the invention

This invention is directed to lubricating fluids suitable for use under extremely low temperature (i.e., —40 to —75° F.) conditions. The invention is directed specifically to synthetic hydrocarbon compositions, and to mixtures of such compositions, having the requisite physical properties for such use.

## GENERAL BACKGROUND

It is known that certain dialkylbenzenes (e.g., those having C<sub>10</sub>—C<sub>15</sub> alkyl groups) have physical properties which render them useful as low temperature lubricants. For example, U.S. Pat. No. 3,173,965 contains such teachings. It is also known that synthetic hydrocarbon lubricants which contain a major amount of di-n-alkylbenzenes, or di-n-long-chain alkaryl, and a minor amount of other hydrocarbon (e.g., diphenylalkanes or trialkyl substituted tetrahydronaphthalenes) have properties which render them useful as low temperature lubricants. U.S. Pat. Nos. 3,288,716; 3,588,739; and 3,662,012 contain such teachings.

The use of linear mono-olefin oligomers as lubricants is also well known. While these materials have outstanding physical properties (e.g., viscosity index and pour point) they are deficient in oxidation stability and compatibility with various conventional lubricating oil additives.

I have discovered that mixtures of di-n-long-chain alkaryl (or synthetic hydrocarbon compositions containing a major amount of di-n-long-chain alkaryl) and linear mono-olefin oligomers have certain unexpectedly improved properties over either alone.

More specifically, the mixtures of dialkaryl and linear mono-olefin oligomers provide the following improvements:

(a) The —40° F. viscosity, as compared to the interpolated viscosity, is lower than that of either material alone;

(b) The mixture is more compatible to additive combinations than the linear mono-olefin oligomers alone;

(c) Compositions comprising the mixture and various additive combinations have improved viscosity indexes as compared to either the dialkaryl or linear mono-olefin oligomers containing the additive package.

## PRIOR ART

A search of the prior art did not produce any reference

showing any advantages of mixtures of di-n-long-chain alkaryl and linear mono-olefin oligomers compared to either material alone. The search did produce thirteen U.S. patents concerned with the general state of the art of the individual materials. In order to make my disclosure complete these patents were the following: 2,190,918; 2,534,095; 3,173,965; 3,518,321; 2,327,705; 2,746,925; 3,436,349; 2,500,165; 3,057,801; 3,449,249; 2,500,244; 3,163,705; and 3,848,857.

## BRIEF SUMMARY OF THE INVENTION

Broadly stated, the present invention is directed to lubricant compositions comprising mixtures of di-n-long-chain alkaryl and linear mono-olefin oligomers.

In one aspect, the invention is directed to lubricant compositions comprising mixtures of linear mono-olefin oligomers and a synthetic hydrocarbon composition containing a major amount of di-n-long-chain alkaryl.

In another aspect, the invention is directed to lubricant compositions comprising a major amount of a mixture of linear mono-olefin oligomers and di-n-long-chain alkaryl and a minor amount of conventional lubricating oil additives.

The relative amounts and nature of the various materials will be described in the detailed description.

## DETAILED DESCRIPTION

One component of the composition of my invention is a di-n-long-chain alkaryl or a synthetic hydrocarbon composition containing a major amount of di-n-long-chain alkaryl.

The term di-n-long-chain alkaryl refers to materials represented by the formula



wherein R and R<sub>1</sub> are alkyl groups containing from 6 to 18 carbon atoms, more suitably from about 9 to about 15 carbon atoms, and preferably from about 10 to about 14 carbon atoms, with the sum of R and R<sub>1</sub> being from about 20 to about 28 carbon atoms and wherein A and A<sub>1</sub> are hydrogen or a C<sub>1</sub> or C<sub>2</sub> alkyl group, but preferably are hydrogen.

Thus the preferred di-n-long-chain alkaryl is a di-n-alkylbenzene wherein the alkyl group contains from about 10 to about 14 carbon atoms.

The alkyl groups are substantially straight-chain (thus the term n-alkaryl) wherein, preferably, at least 95 percent of the alkyl substituents are bonded to the benzene nucleus through a secondary carbon atom of the respective alkyl groups. While we prefer the term "n-alkaryl" other terms such as linear alkaryl or straight-chain alkaryl are equally descriptive.

The first component of my invention also includes synthetic hydrocarbon compositions containing a major amount (i.e., 60 to 90 weight percent) of the di-n-alkaryl, as defined in the foregoing, and a minor amount of other hydrocarbons, such as diphenylalkanes and trialkyl-substituted tetrahydronaphthalenes, having molecular weights corresponding to the di-n-long-chain alkaryl.

A particularly suitable material for the first component is a synthetic hydrocarbon composition having the following composition.

| Component:                                  | Percent by weight |
|---------------------------------------------|-------------------|
| Di-n-long-chain alkaryl                     | 61—92             |
| Trialkyl-substituted tetrahydronaphthalenes | 5—30              |
| Miscellaneous alkyl aromatics:              |                   |
| Less than                                   | 15                |
| Preferably less than                        | 10                |

The composition is also characterized as having the following properties:

Viscosity index ----- 80-116  
 Pour point, °F. ----- -40-80  
 Molecular weight range ----- 350-526  
 Preferably ----- 375-480

The di-n-long-chain alkaryl meet the description provided in the foregoing.

The trialkyl-substituted tetrahydronaphthalenes can be represented by the formula



wherein  $R_1$  and  $R_2$  contain from 1 to about 13 carbon atoms each, with the sum of  $R_1$  and  $R_2$  being from about 6 to about 14 and  $R_3$  and  $R_4$  contain from 1 to about 16 carbon atoms with the sum of  $R_3$  and  $R_4$  being from about 9 to about 17. The alkyl groups,  $R_1$ ,  $R_2$ ,  $R_3$ , and  $R_4$  are straight-chain.

The trialkyl-substituted tetrahydronaphthalenes have the same boiling range as the di-n-alkylbenzenes. In addition, they have approximately the same molecular weight.

This particular synthetic hydrocarbon alkaryl lubricant can be prepared by any of several methods. It can be prepared by alkylating benzene and tetrahydronaphthalene and blending the resulting product. Also, it can be prepared by alkylating a mixture of mono-n-alkylbenzenes and dialkyl-substituted tetrahydronaphthalenes with a suitable alkylating agent. A particularly suitable method of preparing the synthetic hydrocarbon alkaryl lubricant is by the disproportionation of a mono-n-alkyl-benzene-rich feedstock using  $HF-BF_3$ , aluminum bromide or aluminum chloride as the catalyst.

Suitable mono-n-alkylbenzenes are those containing from about 6 to about 18 carbon atoms in the alkyl groups. Preferably, the alkyl groups of the mono-n-alkylbenzenes contain from about 10 to about 15 carbon atoms. The term "n-alkylbenzenes" has been defined in the foregoing.

A particularly suitable method of preparing this latter-described synthetic hydrocarbon lubricant composition is described in U.S. Pat. No. 3,662,012.

The second component of my invention is a linear mono-olefin oligomer or mixture thereof. These materials are usually prepared from  $\alpha$ -olefins using a suitable catalyst and are usually referred to as  $\alpha$ -olefin oligomers. For preparing the  $\alpha$ -olefin oligomers, there is used one or more  $\alpha$ -olefins containing from 6 to 16 carbon atoms, more suitably from 8 to 12 carbon atoms and preferably 10 carbon atoms. The linear mono-olefin oligomer is characterized as containing at least 50 weight percent, more usually at least 60 weight percent, of materials containing 24 to 60 carbon atoms. When the linear mono-olefin oligomer is prepared by oligomerization of  $\alpha$ -olefins containing 8 to 12 carbon atoms preferably the maximum amount of dimer present is 10 weight percent. The linear mono-olefin oligomers can obtain very small amounts (usually less than 5 weight percent) of branched-chain-olefins or di-olefins.

If desired, in order to improve the oxidation stability thereof, the linear mono-olefin oligomers can be treated by any of several known methods, such as hydrogenation or heat treatment. Whether or not the linear mono-olefin oligomers have been treated to improve their oxidation stability does not affect the improvements due to mixtures of linear mono-olefin oligomers and di-n-alkylbenzenes as described herein.

The mixtures forming the composition of my invention can contain from about 10 to about 90 weight percent, more suitably from about 30 to about 85 weight percent,

and preferably from about 50 to about 80 weight percent linear mono-olefin oligomers.

#### USES FOR IMPROVED LUBRICANT COMPOSITIONS OF MY INVENTION

As is readily apparent to those skilled in the art, there are many uses for the lubricant compositions of my invention. They can be used as crankcase lubricants, turbojet aircraft lubricants, turbine lubricants, hydraulic fluids, transmission fluids, combination crankcase and transmission fluids, steering fluids, and instrument lubricants.

While the lubricants of my invention have many uses per se, usually they are used in compounded formulations containing various additives. Examples of additives which can be used include dispersants and detergents, oxidation inhibitors, corrosion inhibitors, viscosity index improvers, antirust agents, and antifoam agents.

In order to disclose the nature of the present invention still more clearly, the following examples, both illustrative and comparative, will be given. It is to be understood that the invention is not to be limited to the specific conditions or details set forth in these examples except insofar as such limitations are specified in the appended claims.

In the examples the test methods were ASTM or other standard tests. The viscosity index was based on measured 100° and 210° F. viscosities.

The percent deviation from interpolated -40° F. viscosity can be explained as follows:

It is common practice in the petroleum industry to use what is known as ASTM viscosity blending paper to interpolate blend viscosities from component viscosities. It is generally observed that at a given temperature lubricant blends obey the relationship

$\ln \ln (K_b + A) = X \ln \ln (K_1 + A) + (1-X) \ln \ln (K_2 + A)$  where  $K_b$  is the kinematic viscosity of the blend in centistokes,  $K_1$  and  $K_2$  are the blend component viscosities,  $A$  is approximately 0.6, and  $X$  is the weight fraction of component one in the blend. This expression is derived from the Walther equation which describes the viscosity-temperature relationship of lubricant blends. ASTM viscosity blending paper as cited above linearly relates blend composition ( $X$ ) to  $\ln \ln (K_b + A)$ . This relationship was used to arrive at an interpolated blend viscosity. The difference between the interpolated and measured blend viscosities divided by the interpolated value is the percent deviation as used herein.

#### EXAMPLE 1

This example illustrates the improvement in -40° F. viscosity of mixtures of linear mono-olefin oligomers and a synthetic hydrocarbon lubricant containing a major amount of di-n-alkylbenzenes.

The linear mono-olefin oligomer was an  $\alpha$ -olefin oligomer which was prepared from decene-1 and contained the following:

| Oligomer | Formula        | Approximate weight, percent |
|----------|----------------|-----------------------------|
| Dimer    | $C_{10}H_{16}$ | 3.0                         |
| Trimer   | $C_{16}H_{32}$ | 42.3                        |
| Tetramer | $C_{20}H_{40}$ | 23.3                        |
| Pentamer | $C_{24}H_{48}$ | 12.05                       |
| Hexamer  | $C_{28}H_{56}$ | 6.0                         |

The synthetic hydrocarbon lubricant was prepared by disproportionation of a predominantly  $C_{12}$ - $C_{13}$  mono-n-alkylbenzene using  $AlCl_3$  as the catalyst. It had the following composition by mass spectrometer:

Vol. percent<sup>1</sup>  
 68  
 Di-n-alkylbenzenes<sup>2</sup> ----- 68  
 Trialkyl-substituted tetrahydronaphthalenes<sup>3</sup> ----- 22.8

<sup>1</sup> Substantially same as weight percent.

<sup>2</sup> Predominantly  $C_{12}$ - $C_{14}$  alkyl groups.

<sup>3</sup> Substantially the same molecular weight as the di-n-alkylbenzenes.

The physical properties of the  $\alpha$ -olefin oligomers ( $\alpha$ -O-O), the synthetic hydrocarbon lubricant (S.H.L.) and various mixtures of the two materials are shown in Table I below.

TABLE I

|                                     | Composition No. |       |       |       |
|-------------------------------------|-----------------|-------|-------|-------|
|                                     | A               | B     | C     | D     |
| S.H.L., percent wt.                 | 100             | 0     | 90    | 80    |
| $\alpha$ -O-O, percent wt.          | 0               | 100   | 10    | 20    |
| Viscosity cs. at—                   |                 |       | 10    |       |
| $-40^{\circ}$ F                     | 9,587           | 6,769 | 8,823 | 8,079 |
| $100^{\circ}$ F                     | 29.77           | 31.95 | 28.97 | 28.45 |
| $210^{\circ}$ F                     | 5.07            | 5.84  | 5.09  | 5.12  |
| Percent deviation from interpolated |                 |       |       |       |
| $-40^{\circ}$ vis.                  |                 |       | -4.3  | -9.0  |
| Viscosity Index                     | 108             | 140   | 116   | 118   |
| Pour point, $^{\circ}$ F            | -60             | 1 -75 | -70   | -60   |

<sup>1</sup> Below -75.

## EXAMPLE 2

This example illustrates the improvement in  $-40^{\circ}$  F. viscosity of mixtures of a di-C<sub>12</sub>-alkylbenzenes and two hydrogenated  $\alpha$ -olefin oligomers prepared from decene-1.

5 and a synthetic hydrocarbon lubricant containing a major amount of di-n-alkylbenzenes.

The linear mono-olefin oligomer was an  $\alpha$ -olefin oligomer which was prepared from decene-1 and contained at least 50 weight percent of oligomers containing 24 to 60 carbon atoms.

The synthetic hydrocarbon lubricant was prepared by disproportionation of a predominantly C<sub>12</sub>-C<sub>13</sub> mono-n-alkylbenzene using AlCl<sub>3</sub> as the catalyst. It had the following composition by mass spectrometer:

|                                                          | Vol. percent <sup>1</sup> |
|----------------------------------------------------------|---------------------------|
| Di-n-alkylbenzenes <sup>2</sup>                          | 69.3                      |
| Trialkyl-substituted tetrahydronaphthalenes <sup>3</sup> | 22.3                      |

<sup>1</sup> Substantially same as weight percent.

<sup>2</sup> Predominantly C<sub>12</sub>-C<sub>14</sub> alkyl groups.

<sup>3</sup> Substantially the same molecular weight as the di-n-alkylbenzenes.

The viscosity properties of the  $\alpha$ -olefin oligomer ( $\alpha$ -O-O), the synthetic hydrocarbon lubricant (S.H.L.) and various mixtures of the two materials are shown in the table below.

TABLE III

| Weight percent                      | 210       | 100         | 0       | -40         | Percent deviation <sup>1</sup> | Viscosity index |
|-------------------------------------|-----------|-------------|---------|-------------|--------------------------------|-----------------|
| $\alpha$ -O-O, 100%                 | 5.92-5.89 | 35.90-35.06 | 882-884 | 8,212-8,365 |                                | 119-121         |
| S.H.L., 100%                        | 4.97-4.98 | 29.03-28.60 | 866-858 | 8,793-8,941 |                                | 105-109         |
| $\alpha$ -O-O, (25%); S.H.L., (75%) | 5.15      | 29.04       | 856     | 8,559       | -1.8                           | 117             |
| $\alpha$ -O-O, (50%); S.H.L., (50%) | 5.39      | 30.40       | 853     | 8,301       | -3.3                           | 123             |
| $\alpha$ -O-O, (75%); S.H.L., (25%) | 5.63-5.65 | 31.81-31.48 | 886-884 | 8,217-8,254 | -2.3                           | 128-132         |
| $\alpha$ -O-O, (80%); S.H.L., (20%) | 5.67      | 31.92       | 856     | 8,245       | -1.8                           | 130             |
| $\alpha$ -O-O, (85%); S.H.L., (15%) | 5.74      | 32.44       | 861     | 8,254       | -1.4                           | 131             |
| $\alpha$ -O-O, (90%); S.H.L., (10%) | 5.82      | 32.54       | 872     | 8,260       | -1.1                           | 135             |
| $\alpha$ -O-O, (95%); S.H.L., (5%)  | 5.89      | 33.11       | 868     | 8,322       | 0                              | 315             |

<sup>1</sup> From Interpolated -40 viscosity.

$\alpha$ -olefin oligomer B contained 37.5% decene-1- trimer 2% decene-1 tetramer.

$\alpha$ -olefin oligomer B contained 37.5% decene-1 trimmer 45 and 62.5% decene-1 tetramer.

The following examples illustrate the advantage of using mixtures of  $\alpha$ -olefin oligomers and a synthetic hydrocarbon lubricant as the base oil in various compounded lubricants.

## EXAMPLE 4

This example illustrates the advantage of using mixtures as a base oil in a hypoid gear oil. The gear oil contained 6.5% of a commercial extreme pressure additive and 93.5 weight percent of the base oil. The synthetic hydrocarbon lubricant (S.H.L.) and  $\alpha$ -olefin oligomer

TABLE IV

| Ratio: Percent S.H.L.: $\alpha$ -O-O | Hypoid gear oil |       |       |       |                           |
|--------------------------------------|-----------------|-------|-------|-------|---------------------------|
|                                      | 100:0           | 75:25 | 50:50 | 25:75 | 0:100                     |
| Kinematic viscosity, cs. at—         |                 |       |       |       |                           |
| $210^{\circ}$ F                      | 5.08            | 5.25  | 5.45  | 5.64  | 5.90                      |
| $100^{\circ}$ F                      | 29.23           | 30.68 | 31.01 | 32.23 | 36.00                     |
| $0^{\circ}$ F                        | 924             | 901   | 893   | 900   | 920*                      |
| $-40^{\circ}$ F                      | 10,328          | 9,623 | 9,331 | 9,060 | 9,809                     |
| Viscosity Index                      | 111             | 113   | 123   | 128   | 118                       |
| Pour point, $^{\circ}$ F             | -65             | -65   | -65   | -70   | -70                       |
| Storage stability: two weeks at—     |                 |       |       |       |                           |
| $150^{\circ}$ F                      | Pass            | Pass  | Pass  | Pass  | Fail, precipitated        |
| $0^{\circ}$ F                        | Pass            | Pass  | Pass  | Pass  | Fail, cloudy precipitated |

\*Sample cloudy when value determined.

( $\alpha$ -O-O-B) and mixtures of the dialkylbenzene and each of the oligomers are shown in Table II below.

60

TABLE II

|                                     | A     | B     | C     | D     |
|-------------------------------------|-------|-------|-------|-------|
| DAB-C <sub>12</sub> , percent wt.   | 100   | 0     | 70.2  | 70.2  |
| $\alpha$ -O-O-A, percent wt.        | 0     | 100   | 29.8  | 0     |
| $\alpha$ -O-O-B, percent wt.        | 0     | 0     | 0     | 29.8  |
| Viscosity index                     | 105   | 123   | 113   | 111   |
| Viscosity cs. at—                   |       |       |       |       |
| $-40^{\circ}$ F                     | 4,446 | 1,611 | 2,994 | 4,994 |
| $100^{\circ}$ F                     | 20.65 | 14.57 | 18.39 | 23.26 |
| $210^{\circ}$ F                     | 4.06  | 3.43  | 3.86  | 4.44  |
| Percent deviation from interpolated |       |       |       |       |
| $-40^{\circ}$ vis.                  |       |       | -7.5  | -5.0  |
| Pour point, $^{\circ}$ F            | -75   | -75   |       |       |

## EXAMPLE 3

This example illustrates the improvement in  $-40^{\circ}$  F. viscosity of mixtures of linear mono-olefin oligomers 75

( $\alpha$ -O-O) were the same as in Example 3. The results are shown in Table IV.

## EXAMPLE 5

65 This example illustrates the advantages of using mixtures as a base oil in a gas turbine oil. The turbine oil contained 6.53 weight percent of an additive combination which comprised a friction and antiwear compound, an antioxidant, a viscosity control polymer, and a corrosion inhibitor and 93.48 weight percent of the base oil. The synthetic hydrocarbon lubricant (S.H.L.) and  $\alpha$ -olefin oligomer ( $\alpha$ -O-O) were the same as in Examples 3 and 4. The results are shown in Table V.

TABLE V

| Ratio: Percent S.H.L.: Percent $\alpha$ -O-O | Gas turbine oil |       |              |                            |                            |
|----------------------------------------------|-----------------|-------|--------------|----------------------------|----------------------------|
|                                              | 100:0           | 75:25 | 50:50        | 25:75                      | 0:100                      |
| Kinematic viscosity, cs. at—                 |                 |       |              |                            |                            |
| 210° F.                                      | 5.33            | 5.50  | 5.68         | 5.81                       | (1).                       |
| 100° F.                                      | 30.34           | 30.69 | 31.16        | 31.97                      |                            |
| 0° F.                                        | 949             | 911   | 904          | 1,012                      |                            |
| —40° F.                                      | 10,452          | 9,718 | 9,439        | 11,027                     |                            |
| Viscosity index                              | 120             | 129   | 136          | 138                        | (1).                       |
| Pour point, ° F.                             | —65             | —65   | —70          | —70                        | (1).                       |
| Storage stability; two weeks at—             | Pass            | Pass  | Pass         | Pass                       | Fail, precipitated.        |
| 150° F.                                      |                 |       |              |                            |                            |
| 0° F.                                        | Pass            | Pass  | Fail, cloudy | Fail, cloudy, precipitated | Fail, cloudy precipitated. |

<sup>1</sup> Not run, sample precipitated.<sup>2</sup> Sample cloudy when value determined.

## EXAMPLE 6

This example is both illustrative and comparative in showing the effect of using mixtures as a base oil in an S.E. engine oil. Use of the mixtures gave an improvement in viscosity index but no improvement in compatibility to the additive package. The engine oil contained 7.95 weight percent of an additive combination which comprised an ashless dispersant, an overbased magnesium sulfonate, a zinc dithiophosphate inhibitor, an overbased calcium phenate, and an ashless antioxidant and 92.05 weight percent of the base oil. The synthetic hydrocarbon lubricant (S.H.L.) and  $\alpha$ -olefin oligomer ( $\alpha$ -O-O) were the same as in Examples 3, 4 and 5. The results are shown in Table VI.

TABLE VI

| Ratio: percent S.H.L.: percent $\alpha$ -O-O | S.E. engine oil |       |       |       |       |
|----------------------------------------------|-----------------|-------|-------|-------|-------|
|                                              | 100:0           | 75:25 | 50:50 | 25:75 | 0:100 |
| Kinematic viscosity, cs. at—                 |                 |       |       |       |       |
| 210° F.                                      | 6.02            | 6.25  | 6.46  | 6.72  | 7.07  |
| 100° F.                                      | 36.89           | 37.47 | 38.69 | 40.11 | 45.29 |
| 0° F.                                        | 1,209           | 1,194 | 1,191 | 1,204 | 1,229 |
| —30° F.                                      | 6,719           | 6,546 | 6,405 | 6,340 | 6,447 |
| Viscosity index                              | 119             | 127   | 130   | 135   | 126   |
| Pour point, ° F.                             | —65             | —60   | —65   | —65   | —65   |
| Storage stability; two weeks at—             | Pass            | Pass  | Pass  | Pass  | Pass  |
| 150° F.                                      |                 |       |       |       |       |
| 0° F.                                        | Pass            | Pass  | Pass  | Pass  | Pass  |

<sup>1</sup> Sample cloudy when value determined.

## EXAMPLE 7

This example illustrates the improvement in —40° F. viscosity of mixtures of linear mono-olefin oligomers and a di-n-C<sub>10</sub>-alkylbenzene.

The linear mono-olefin oligomer was prepared from decene-1 and contained at least 50 weight percent of oligomers containing 24–60 carbon atoms.

The di-n-C<sub>10</sub>-alkylbenzene had the following composition, as determined by mass spectrometer:

|                               | Percent |
|-------------------------------|---------|
| Didecylbenzenes               | 96.4    |
| Tridecylbenzenes              | 2.9     |
| Miscellaneous alkyl aromatics | 0.6     |

The viscosity properties of the  $\alpha$ -olefin oligomer ( $\alpha$ -O-O) and the di-n-C<sub>10</sub>-alkylbenzene (DAB-C<sub>10</sub>) and various mixtures of the two are shown in Table VII.

TABLE VII

| Ratio: percent $\alpha$ -O-O: percent DAB-C <sub>10</sub> (by weight) | 100:0 90:10 80:20 60:40 40:60 20:80 10:90 0:100 |       |       |       |       |       |       |       |  |
|-----------------------------------------------------------------------|-------------------------------------------------|-------|-------|-------|-------|-------|-------|-------|--|
|                                                                       | 5.90                                            | 5.60  | 5.23  | 4.65  | 4.16  | 3.71  | 3.49  | 3.33  |  |
| Measured kinematic viscosity at—                                      |                                                 |       |       |       |       |       |       |       |  |
| 210° F.                                                               | 5.90                                            | 5.60  | 5.23  | 4.65  | 4.16  | 3.71  | 3.49  | 3.33  |  |
| 100° F.                                                               | 33.25                                           | 30.41 | 27.90 | 24.00 | 20.57 | 17.79 | 16.49 | 15.45 |  |
| —40° F.                                                               | 7,949                                           | 7,269 | 6,485 | 4,997 | 4,058 | 3,345 | 3,049 | 2,867 |  |
| Linearly interpolated kinematic viscosity cs. at—                     |                                                 |       |       |       |       |       |       |       |  |
| 210° F.                                                               | 5.65                                            | 5.39  | 4.88  | 4.36  | 3.85  | 3.59  |       |       |  |
| 100° F.                                                               | 31.5                                            | 29.7  | 26.1  | 22.5  | 19.0  | 17.3  |       |       |  |
| —40° F.                                                               | 7,450                                           | 6,940 | 5,910 | 4,900 | 3,880 | 3,370 |       |       |  |
| Percent deviation from interpolated viscosity at—                     |                                                 |       |       |       |       |       |       |       |  |
| 210° F.                                                               | 0.9                                             | 3.0   | 4.7   | 4.6   | 3.6   | 2.8   |       |       |  |
| 100° F.                                                               | 3.5                                             | 6.1   | 8.0   | 8.4   | 6.3   | 4.6   |       |       |  |
| —40° F.                                                               | 2.4                                             | 6.5   | 15.4  | 17.1  | 13.6  | 9.5   |       |       |  |
| Viscosity index                                                       | 134                                             | 133   | 132   | 126   | 120   | 106   | 97    | 92    |  |

The data in Table VII shows that the measured —40° F. viscosity is lower (which is an improvement) than the interpolated viscosity for all of the mixtures and particularly is better for the blends containing 60, 40, and 20% of the oligomers. For example, on the blend containing 40% oligomers, the measured —40° F. viscosity was 4058 cs., while the interpolated viscosity was 4900 cs. Thus the measured viscosity showed a 17.1% deviation (an improvement) over the measured viscosity.

While we have defined previously what is meant by interpolated viscosity, the following amplification of the definition is provided. Referring to the table, it will be observed that —40° F. viscosities for the pure materials were as follows: olefin oligomer—7949; di-C<sub>10</sub>-alkylbenzene—2867.

The interpolated —40° F. viscosity for various mixtures of the two materials was determined by interpolation of these values using ordinary graph paper, whereas logarithmic graph paper was used in the other examples herein. This difference in type of graph paper does not make a substantial difference for the values described herein.

Thus, having described the invention in detail, it will be understood by those skilled in the art that certain variations and modifications may be made without departing from the spirit and scope of the invention as defined herein and in the appended claim.

## I claim:

1. A lubricant composition comprising a mixture of about 30 to about 85 weight percent of a first component which is a linear mono-olefin oligomer, or mixtures thereof, and about 15 to about 70 weight percent of a second component which is a di-n-C<sub>10</sub>–C<sub>14</sub> alkylbenzene, a mixture of di-n-C<sub>10</sub>–C<sub>14</sub> alkylbenzenes or a synthetic hydrocarbon composition containing a major amount of di-n-C<sub>10</sub>–C<sub>14</sub> alkylbenzenes, said linear mono-olefin oligomer, or mixtures thereof, containing at least 60 weight percent oligomers which contain 24 to 60 carbon atoms.

2. The lubricant composition of claim 1 wherein said linear mono-olefin oligomers is prepared from  $\alpha$ -olefins containing 8 to 12 carbon atoms.

3. The lubricant composition of claim 2 wherein the second component is a synthetic hydrocarbon composition having the following composition:

Component: Percent by weight  
 Di-n-C<sub>10</sub>-C<sub>14</sub> alkylbenzenes ----- 61-92  
 Trialkyl-substituted tetrahydronaphthalenes - 5-30  
 Miscellaneous alkyl aromatic compounds --- <15

said synthetic hydrocarbon composition being characterized as having a molecular weight of about 375 to about 480, said trialkyl-substituted tetrahydronaphthalenes being represented by the formula



wherein R<sub>1</sub> and R<sub>2</sub> are straight-chain alkyl groups containing from 1 to about 13 carbon atoms each, with the sum of R<sub>1</sub> and R<sub>2</sub> being from about 6 to about 14, and wherein R<sub>3</sub> and R<sub>4</sub> are straight-chain alkyl groups containing from about 1 to about 16 carbon atoms, with the sum of R<sub>3</sub> and R<sub>4</sub> being from about 9 to about 17.

4. The lubricant composition of claim 1 wherein the amount of said first component is about 50 to about 80 weight percent and the amount of said second component is about 20 to about 50 weight percent.

5. The lubricant composition of claim 3 wherein the amount of said first component is about 50 to about 80 weight percent and the amount of said second component is about 20 to about 50 weight percent.

6. A lubricant composition comprising a mixture of about 10 to about 90 weight percent of a first component which is a linear mono-olefin oligomer, or mixtures thereof, said linear mono-olefin oligomer containing at least 50 weight percent oligomer, which contain 24 to 60 carbon atoms, and about 10 to about 90 weight percent of a second component which is a di-n-long-chain alkaryl compound, a mixture of di-n-long-chain alkaryl compounds, or a synthetic hydrocarbon composition containing a major amount of di-n-long-chain alkaryl compounds, said lubricant composition being characterized in that:

(a) said di-n-long-chain alkaryl compound is represented by the formula



wherein R and R<sub>1</sub> are substantially straight-chain alkyl groups containing from 6 to 18 carbon atoms, with the sum of R and R<sub>1</sub> being from about 20 to about 28 carbon atoms and wherein A and A<sub>1</sub> are hydrogen or a C<sub>1</sub> or C<sub>2</sub> alkyl group, and

(b) said synthetic hydrocarbon composition has the following composition:

Component: Percent by weight  
 Di-n-long-chain alkaryl ----- 61-92  
 Trialkyl-substituted tetrahydronaphthalenes ----- 5-30  
 Miscellaneous alkyl aromatic compounds ----- <15

said synthetic hydrocarbon composition being characterized as having a molecular weight range of about 350 to about 526, said di-n-long-chain alkaryl being represented by the formula



wherein R and R<sub>1</sub> are substantially straight-chain alkyl groups containing from 6 to 18 carbon atoms, with the sum of R and R<sub>1</sub> being from about 20 to about 28 carbon atoms, and wherein A and A<sub>1</sub> are hydrogen or a C<sub>1</sub> or C<sub>2</sub> alkyl group, said trialkyl substituted tetrahydronaphthalenes being represented by the formula



wherein R<sub>1</sub> and R<sub>2</sub> are straight-chain alkyl groups containing from 1 to about 13 carbon atoms each, with the sum of R<sub>1</sub> and R<sub>2</sub> being from about 6 to about 14, and wherein R<sub>3</sub> and R<sub>4</sub> are straight-chain alkyl groups containing from about 1 to about 16 carbon atoms, with the sum of R<sub>3</sub> and R<sub>4</sub> being from about 9 to about 17.

7. The lubricant composition of claim 6 wherein said linear mono-olefin oligomer is prepared from  $\alpha$ -olefins containing 6 to 16 carbon atoms.

8. The lubricant composition of claim 7 wherein the alkyl groups R and R<sub>1</sub> contain from about 9 to about 15 carbon atoms.

9. The lubricant composition of claim 8 wherein R and R<sub>1</sub> contain from about 10 to about 14 carbon atoms.

10. The lubricant composition of claim 9 wherein A and A<sub>1</sub> are hydrogen.

11. A lubricant composition of claim 10 wherein said linear mono-olefin oligomer is prepared from  $\alpha$ -olefins containing 8 to 12 carbon atoms.

#### References Cited

##### UNITED STATES PATENTS

|    |           |        |                |       |          |
|----|-----------|--------|----------------|-------|----------|
| 55 | 3,322,848 | 5/1967 | Garwood et al. | ----- | 252-59 X |
|    | 3,598,739 | 8/1971 | Sias           | ----- | 252-59 X |
|    | 3,642,634 | 2/1972 | Olund          | ----- | 252-59 X |

WARREN H. CANNON, Primary Examiner